# EUROPEAN PATENT SPECIFICATION

(11) **EP 1 993 108 B1**
(45) Date of publication and mention of the grant of the patent: **01.03.2017**
(21) Application number: 07108464.4
(22) Date of filing: 18.05.2007
(51) Int. Cl.: H01C 7/105, H01C 7/108, H01C 7/112, H01C 7/115, H01C 7/118

(54) **Material composition having a core-shell microstructure used for a varisator**
Für einen Varistor verwendete Materialzusammensetzung mit Kern-Schalen-Mikrostruktur
Composition de matériau doté d'une microstructure noyau-enveloppe utilisé pour un varistor

(43) Date of publication of application: 19.11.2008
(73) Proprietor: Bee Fund Biotechnology Inc., Taoyuan County (TW)
(72) Inventor: Lien, Ching-Hohn, 333, Guishan Shiang, Taoyuan County (TW); Kuo, Chen-Tsung, Banqiao City, Taipei County (TW); Lin, Jun-Nan, Zhubei City, Hsinchu County (TW); Zhu, Jie-An, 333, Guishan Shiang, Taoyuan County (TW); Zhang, Li-Yun, 333, Guishan Shiang, Taoyuan County (TW); Lien, Wei-Chang, Taipei (TW)
(74) Representative: Beck, Michael Rudolf

(56) References cited:
- EP-A1- 0 115 050
- US-A- 3 725 836

## Description

### BACKGROUND OF THE INVENTION

### 1. Field of the Invention

The present invention relates to a powderized material composition for a varistor according to the preamble portion of claim 1; and a method for manufacturing a varistor from said powedrized material composition.

### 2. Description of the Related Art

In the electronic industry, the current trend is towards higher operational frequency and smaller volume. Thus, varistors or surge absorbers are conventionally used in high-frequency applications for protecting IC from getting damaged due to overvoltage.

Various materials, such as SrTiO₃, SiC, ZnO, Fe2O₃, SnO₂, TiO₂, BaTiO₃ and Diode, may be implemented to absorb surge. However, since the materials present diverse characteristics in surge absorbent abilities, static absorbent abilities and other properties, not all of the mentioned materials can be applied in manufacture and practical applications.

A silicon diode provides surge absorbent ability relying on the PN interface. A varistor made from this material disadvantageously possesses relatively higher breakdown voltage and inferior surge absorbent ability.

Varistors constructed of Fe₂O₃ and BaTiO₃ have the surge absorbent ability relying on the interface between electrodes and ceramics. However, such varistors present inferior electrical properties and are unsuitable for making high-voltage components.

The surge absorbent ability of varistors made from ZnO, TiO₂, SnO₂ or SrTiO₃ typically depends on the interface between semi-conductive grains and grain-boundary insulating layers. However, the grain-boundary insulating layers are primarily composed of crystalline phases, such as crystalline phases of α-Bi₂O₃, Na₂O or SrTiO₃. Thus, the disadvantage of such varistors is that the production of the grain-boundary insulating layers requires sintering at a relatively higher temperature.

US 3,725,836 teaches making a varistor paste by dispersing a uniform mixture of glass frit powder and zinc oxide powder in a liquid vehicle. The liquid vehicle is removed in an electric furnace so that the glas frit fuses so as to bond the zinc oxide powder particles and to adhere firmly to an insulating base. In other words, US 3,725,836 teaches two separate powder components that are mixed with each other to form a varistor layer. It is therefore not possible to control the distance between zinc oxide grains in the resulting ceramic.

US 3 725 836 A1 and EP 0 115 050 A1 describe varistor materials according to claim 1.

### SUMMARY OF THE INVENTION

The present invention, which is defined by the features of the independent claims, has been accomplished under these circumstances in view. It
is the objective of the present invention to provide a novel material composition for a varistor.

This technical problem is solved by the powderized material composition as defined in claim 1. Advantageous embodiments are indicated in further claims.

The disclosed material composition has a core-shell microstructure at least comprising a cored-structure made of a conductive or semi-conductive material and a shelled-structure made from a glass material to wrap the cored-structure.

Particularly, varistors constructed from the disclosed material composition can be produced through sintering the material composition at a relatively lower temperature, which is typically between 600°C and 1,100°C. Besides, the electrical properties of such varistors can be decided and designated through adjusting some particular parameters such as the size and properties of the grain of the cored-structure, the thickness and insulation resistance of the insulating layer of the shelled-structure, and the interval between two parallel electrodes and the overlap area of the electrode materials of the varistors.

The novel material composition can be used for making both single-layered varistors and multiple-layered varistors, and the electrical properties of the varistors can be decided and designated during manufacturing for meeting various practical needs.

Further, the present invention can be used for manufacturing varistors with desired voltage. The method comprises sintering a novel material composition having a core-shell microstructure at a relatively lower temperature. In sintering at lower temperature, since the shelled-structure of the novel material composition is made from a glass material which has almost no reaction with the material of the cored-structure of the material composition, electrical properties of such varistors can be decided and designed by precisely controlling the size and properties of the grain of the cored-structure, the thickness and insulation resistance of the insulating layer of the shelled-structure, and the interval between two parallel electrodes and the overlap area of the electrode materials of the varistors.

### BRIEF DESCRIPTION OF THE DRAWINGS

Fig. 1 is a schematic drawing of a varistor constructed of a novel material composition having a core-shell microstructure of the present invention.

### DETAILED DESCRIPTION OF THE PREFERRED EMBODIMENT

As shown in Fig. 1, the disclosed material composition 11 of the present invention has a core-shell microstructure which at least comprises a shelled-structure 12 and a cored-structure 14 wrapped by the shelled-structure 12.

In particular, the cored-structure 14 of the core-shell microstructure of the material composition 11 is made of a conductive or semi-conductive material, and the shelled-structure 12 of the core-shell microstructure is made from a glass material that wraps the cored-structure 14.

The material composition 11 of the present invention may be in application of being manufactured into a ceramic component 20 for a varistor 10 through a standard ceramic processing.

The conductive material used as the cored-structure 14 of the core-shell microstructure of the material composition 11 of the present invention can be one of, a combination of two or more of or a combination of alloys of the metals selected from the group containing Fe, Al, Ni, Cu, Ag, Au, Pt and Pd.

The semi-conductive material used as the cored-structure 14 of the core-shell microstructure of the material composition 11 of the present invention can be one of, or a combination of two or more of the metals selected from the group containing ZnO, SrTiO₃, BaTiO₃, SiC, TiO₂, SnO₂, Si and GaAs.

The cored-structure 14 of the core-shell microstructure of the material composition 11 of the present invention can alternatively be made with a combination of the aforementioned conductive materials and semi-conductive materials.

The glass material used as the shelled-structure 12 of the core-shell microstructure of the material composition 11 of the present invention can be selected from the group containing silicate glass, boron glass, alumina-silica glass, phosphate glass and lead glass.

Referred to Fig. 1, the material composition 11 of the present invention can be used to manufacture a varistor 10 which provides outstanding electrical properties through the manufacturing steps described below.
1. Firstly, a proper metal conductor, a semi-conductive metallic oxide or a general semi-conductive material is suitably selected and soaked into a sol-gel having the formula containing silicate glass, boron glass, lead glass or phosphate glass. Thus, as a result of heterogeneous precipitation, the surface of the grain of the metal conductor or semi-conductive material can be wrapped by a layer of the material containing glass.
   Then the resultant of core-shell combination is sintered at the temperature between 500°C and 900°C for 0.5 to 8 hours so that the layer of the inorganic or organic material containing glass wrapped around the surface of the conductor or the semi-conductive material can be turned in to a glass layer. By this way, a powderized material composition 11 of the present invention having a core-shell microstructure constructed of a cored-structure 14 wrapped by a shelled-structure 12 is realized.
2. For manufacturing a single-layered varistor 10, a lot of sintered and powderized material compositions 11 are mixed with appropriate binder and dispersant and formed under a forming pressure of 10000 lb/in² (psi). After a debinding process, the formation is sintered at a temperature between 600°C and 1,100°C for 0.5 to 4 hours to get a sintered ceramic body 20. Then the sintered ceramic body 20 is smeared with conductive silver paste at the upper and lower surface thereof and treated at a temperature between 500°C to 800°C as reduction process. Thereby, a single-layered varistor 10 of Fig. 1 is realized.
3. For manufacturing a multiple-layered varistor 10, a lot of sintered and powderized material compositions 11 are mixed with appropriate binder, dispersant, plasticizer and organic solvent to form a paste material having the formulated powders. Then doctor blade casting is conducted with the paste to make a green tape wherein the thickness of the green tape is made between 15µm and 200µm by adjusting the parameters such as the viscosity of the paste and the thickness of the blade during making the green tape.
   Afterward, the green tape is cut into pieces with a predetermined size, and then, either a precious metal selected from one of the group containing platinum, silver, palladium, gold and rhodium or an alloy composed of any two of the precious metals is printed onto the pieced green tape as an inner electrode 21. Several pieces of the printed green tape are stacked in the manner that the ends of the inner electrodes alternately appear. After being covered by an upper lid and a lower lid and undergoing pressure equalization, the stack of the pieces is then cut at predetermined positions into green grains.
   The green grains are further sintered in a sintering furnace at a temperature between 600°C and 1,100°C for 0.5 to 4 hours. Then at two ends of the sintered grains, where the inner electrodes 21 appear, are respectively formed as an outer electrode 22 after being coated with silver (Ag). The aforesaid composition is finally reduced at a temperature between 500°C and 900°C to realize the multiple-layered varistor 10.
4. At last, the basic electrical properties of the single-layered or multiple-layered varistor 10, including breakdown voltage (V1mA), nonlinear exponent (α), leakage current (iL), ESD tolerance and restraining voltage, are measured. And, the definition of ESD tolerance is that when the varistor 10 receives a static electricity the highest surge current is measured from the displacement of breakdown voltage is occurred within ±10% after the highest inrush current.

### Preferred Embodiments

The following Examples 1 through 5 are provided to demonstrate that the disclosed material composition 11 of the present invention is adaptable to manufacture a varistors 10 having several outstanding electrical properties.

Moreover, the present invention further provides a method for manufacturing a varistor whose voltage can be designated as needed. The varistor 10 is constructed of a material composition 11 having a core-shell microstructure which at least comprises a cored-structure 14 wrapped by a shelled-structure 12.

The varistor 10 is made by sintering the material composition 11 at a relatively lower temperature. In the lower temperature sintering, since shelled-structure 12 made from a glass material has almost no reaction with the material of cored-structure 14, the electrical properties of such varistors 10 can be decided and designated by precisely controlling the size and properties of the grain of cored-structure 14, the thickness and insulation resistance of the insulating layer of the shelled-structure 12, of the interval between two parallel electrodes 21 and the overlap area of the electrodes 21 of the varistors 10.

### Example 1

Silicon carbide powders sized between 0.6µm and 1.0µm are selected and soaked into a transparent organic solution primarily containing ethyl silicate. Trough pH control of the solution, glass containing in the composition can be evenly precipitated on the surface of the silicon carbide powders. Then the powders are dried and sintered at 600°C for 2 hours so that the silicon carbide powders coated with silicate glass can be obtained.

The sintered powders are mixed with appropriate binder, dispersant, plasticizer and organic solvent to form an organic paste. The viscosity of the paste is carefully controlled to facilitate the control of the thickness of the green tape to be made. Then doctor blade casting is conducted with the paste to make a green tape wherein the thickness of the green tape is made to 15∼200µm. Afterward, 6 layers of the green tape printed with inner electrodes are stacked in the manner that the inner electrodes alternately appear. For reducing the leakage current and enhancing the stability of the product, the resultant construction is added at the upper and lower end respectively with 5 layers of tape whereon no electrode is printed. The construction is compacted at 70°C and 3000 lb/in² (psi) and cut at predetermined positions into green grains.

The green grains are further sintered in a sintering furnace at 900°C for 2 hours. Then the sintered grains are coated with silver paste at the appearing end of the inner electrodes and further treated at 800°C for 0.5 hour. Thereby, a multiplayer varistor 10 of Fig. 1 sized 1.0 x 0.5 x 0.5 is obtained.

At last, the basic electrical properties of the varistor 10, including breakdown voltage (V1mA), nonlinear exponent (α), leakage current (iL), ESD tolerance and restraining voltage are measured to determine the practicability of the varistor 10.

The measured results are shown in Table 1 and Table 2, wherein Table 1 describes the effect of the amount of the glass on the properties of the varistor 10. According to the results of samples 1 to 5, the larger amount of the glass leads the higher breakdown voltage (V1mA), the higher nonlinear exponent (α) and the lower leakage current (iL) of the varistor 10.

When the amount of glass is greater than 20%, the leakage current (iL) of the varistor 10 is reduced to a relatively lower level and can pass the electrostatic discharge immunity test of 8KV.

**Table 1**

| Sample | Glass Percentage (%) | Thickness of the tape (µm) | V1mA(V) | α | iL (µA) | ESD Tolerence (8KV) |
|---|---|---|---|---|---|---|
| 1 | 10 | 50 | 105.4 | 5.57 | 200.2 | NG |
| 2 | 20 | 50 | 123.7 | 7.59 | 79.0 | Pass |
| 3 | 30 | 50 | 235.1 | 15.08 | 67.9 | Pass |
| 4 | 50 | 50 | 378.1 | - | 9.2 | Pass |
| 5 | 70 | 50 | 676.0 | - | 0.2 | Pass |

Table 2 shows the electrical properties of the varistors 10 made from different thickness of the green tapes sintered at 900°C. It is observed that the breakdown voltages (V1mA) of the varistors 10 are proportioned to the thickness of the green tapes. The thicker the green tape is, the higher breakdown voltage (V1mA) of the resultant varistor 10 has.

**Table 2**

| Sample | Thickness of the tape (µm) | V1mA(V) | α | iL (µA) | ESD Tolerence (8KV) |
|---|---|---|---|---|---|
| 6 | 20 | 80.4 | 11.78 | 63.5 | Pass |
| 7 | 35 | 147.2 | 13.62 | 57.8 | Pass |
| 8 | 50 | 235.1 | 15.08 | 67.9 | Pass |
| 9 | 70 | 301.2 | 14.88 | 62.3 | Pass |

Through the above Tables 1 and 2, it is learned that through controlling the amount of glass and thickness of the green tape, a multiple-layered varistor 10 can be manufactured with designated voltage.

### Example 2

In the present example, semi-conductive strontium titanate powders are implemented as the material of the cored-structure of the previous Example 1, while boron glass is used as the material of the shelled-structure. Similarly, the semi-conductive strontium titanate powders are coated with the boron glass and the chip component fabrication is conducted. Then doctor blade casting is conducted to make a green tape of 50µm thickness and the green tape is made into green grains each having two layers of inner electrodes. The construction is sintered at 850°C for 2 hours to obtain a multiple-layered varistor 10.

The varistor 10 has electrical properties as shown in Table 3 and can pass the electrostatic discharge immunity test of 8KV.

**Table 3**

| Sample | Thickness of the tape (µm) | V1mA(V) | α | iL (µA) | ESD Tolerence (8KV) |
|---|---|---|---|---|---|
| 10 | 50 | 261.8 | 8.76 | 2.9 | Pass |

### Example 3

In the present example, metal nickel powders are implemented as the material of the cored-structure of the previous Example 1, while silicate glass is used as the material of the shelled-structure. Similarly, the metal nickel powders are coated with the silicate glass and the chip component fabrication is conducted. Then doctor blade casting is conducted to make a green tape of 30µm thickness and the green tape is made into green grains each having two layers of inner electrodes. The construction is sintered at 800°C for 2 hours to obtain a multiple-layered varistor 10.

The varistor 10 has electrical properties as shown in Table 4 and can pass the electrostatic discharge immunity test of 8KV.

**Table 4**

| Sample | Thickness of the tape (µm) | V1mA(V) | α | iL (µA) | ESD Tolerance (8KV) |
|---|---|---|---|---|---|
| 11 | 30 | 241.8 | - | 1.22 | Pass |

### Example 4

In the present example, metal copper powders are implemented as the material of the cored-structure of the previous Example 1, while silicate glass is used as the material of the shelled-structure. Similarly, the metal copper powders are coated with the silicate glass and the chip component fabrication is conducted. Then doctor blade casting is conducted to make a green tape of 50µm thickness and the green tape is made into green grains each having two layers of inner electrodes. The construction is sintered at 700°C for 2 hours to obtain a multiple-layered varistor 10.

The varistor 10 has electrical properties as shown in Table 5 and can pass the electrostatic discharge immunity test of 8KV.

**Table 5**

| Sample | Thickness of the tape (µm) | V1mA(V) | α | iL (µA) | ESD Tolerance (8KV) |
|---|---|---|---|---|---|
| 12 | 50 | 548.5 | - | 0.67 | Pass |

### Example 5

The research is now directed to the effect of the size of the material on the electrical properties of the components. Differently sized SiC powders ranged from 0.5 to 10µm are taken as the cored-structure of the previous Example 1. Then the powders are relatively coated with glass and the chip component fabrication is conducted. Then doctor blade casting is conducted to make green tapes of 50µm thickness and general multiple-layered chip components are obtained.

The electrical properties of the components are listed in Table 6 in which it can be found that the breakdown voltage (V1mA) of the component is related to the original powder size of the cored-structure. When the cored-structure has a smaller size, the resultant component possesses a lower breakdown voltage (V1mA).

**Table 6**

| Sample | Thickness of the tape (µm) | V1mA(V) | α | iL (µA) | ESD Tolerance (8KV) |
|---|---|---|---|---|---|
| 13 | 10.0 | 285.1 | 17.58 | 26.8 | Pass |
| 14 | 2.5 | 254.3 | 17.24 | 27.9 | Pass |
| 15 | 0.8 | 230.6 | 16.04 | 28.6 | Pass |

Although a particular embodiment of the invention has been described in detail for purposes of illustration, it will be understood by one of ordinary skill in the art that numerous variations will be possible to the disclosed embodiments without going outside the scope of the invention as disclosed in the claims.

## Claims

1. A powderized material composition (11) for a varistor (10), comprising:
a metal conductor, a semi-conductive metallic oxide or semi-conductive material; and
a glass material;
**characterized in that**
the powderized material composition has a core-shell microstructure wherein a grain forming a cored-structure (14) is made of said metal conductor, semi-conductive metallic oxide or semi-conductive material and a shelled-structure (12) wrapped around the surface of the grain of the cored-structure (14) to form an insulating layer is made from said glass material.

2. The material composition as defined in claim 1, wherein the metal conductor is one or a combination of two or more or a combination of alloys of the metals selected from the group containing Fe, Al, Ni, Cu, Ag, Au, Pt and Pd.

3. The material composition as defined in claim 1, wherein the semi-conductive material is one or a combination of two or more selected from the group containing ZnO, SrTiO₃, BaTiO₃, SiC, TiO₂, SnO₂, Si and GaAs.

4. The material composition as defined in one of claims 1, wherein the glass material is selected from the group containing silicate glass, boron glass, alumina-silica glass, phosphate glass and lead glass.

5. A method for manufacturing a varistor from the powderized material composition (11) of claim 1, wherein the varistor (10) is made through sintering the material composition (11) at a temperature between 600°C and 1,100°C, and wherein the breakdown voltage of the varistor (10) is adjusted by precisely controlling the size of the grain of the cored-structure (14) and/or controlling the thickness or insulation resistance of the shelled-structure (12) forming the insulating layer.

6. The method of claim 5 for manufacturing a multiple-layered varistor (10) comprising:
a) selecting powderized material compositions (11) as raw material, each containing a core-shell microstructure wherein a grain forming a cored-structure (14) is made of a conductive or semi-conductive material and shelled-structure (12) wrapped around the surface of the grain of the cored-structure (14) to form an insulating layer is made of glass material;
b) mixing said powderized material compositions (11) with appropriate binder, dispersant, plasticizer and organic solvent to form a paste material;
c) producing a green tape made of the paste material through doctor blade casting;
d) stacking a predetermined number of green tapes having an inner electrode (21) printed thereon in such a manner that ends of the inner electrodes (21) alternately appear;
e) sintering the stacked green tapes at a temperature between 600°C and 1,100°C,
f) wherein the breakdown voltage of the varistor (10) is designed
at step a) by precisely controlling either the size of the cored-structure (14) or the thickness of the glass layer of the shelled-structure (12) of the powderized material compositions (11), and/or
at step c) by precisely controlling the thickness of each green tape within a range between 15µm and 200µm.

7. A multiple-layered varistor (10) produced by the method of claim 6, wherein in a sintered ceramic body (20) constructed from the powderized material compositions (11) contains an amount of glass greater than 20%.

8. The multiple-layered varistor (10) as defined in claim 7, wherein the conductive material is selected from the group consisting of Fe, Al, Ni, Cu, Ag, Au, Pt, Pd and alloy thereof, and the semi-conductive material is selected from the group consisting of ZnO, SrTiO₃, BaTiO₃, SiC, TiO₂, SnO₂, Si and GaAs.

## Patentansprüche

1. Pulverförmige Materialzusammensetzung (11) für einen Varistor (10), umfassend:
einen Metallleiter, ein halbleitendes Metalloxid oder halbleitendes Material; und
ein Glasmaterial;
**dadurch gekennzeichnet, dass**
die pulverförmige Materialzusammensetzung eine Kern-Schalen-Mikrostruktur aufweist, wobei ein Korn, das eine Kernstruktur (14) bildet, aus dem Metallleiter, dem halbleitenden Metalloxid oder dem halbleitenden Material besteht und eine Schalenstruktur (12), die um die Oberfläche des Korns der Kernstruktur (14) gehüllt ist, um eine Isolationsschicht zu bilden, aus dem Glasmaterial besteht.

2. Materialzusammensetzung nach Anspruch 1, wobei der Metallleiter eines oder eine Kombination aus zwei oder mehr oder eine Kombination aus Legierungen aus Metallen ist, die aus der Gruppe gewählt werden, welche Fe, Al, Ni, Cu, Ag, Au, Pt und Pd enthält.

3. Materialzusammensetzung nach Anspruch 1, wobei das halbleitende Material eines oder eine Kombination aus zwei oder mehreren Materialien ist, die aus der Gruppe gewählt werden, die ZnO, SrTiO₃, BaTiO₃, SiC, TiO₂, SnO₂, Si und GaAs enthält.

4. Materialzusammensetzung nach Anspruch 1, wobei das Glasmaterial aus der Gruppe gewählt wird, die Silikatglas, Borglas, Tonerde-Quarzglas, Phosphatsglas und Bleiglas enthält.

5. Herstellungsverfahren für einen Varistor aus der pulverförmigen Materialzusammensetzung (11) nach Anspruch 1, wobei der Varistor (10) durch Sintern der Materialzusammensetzung (11) bei einer Temperatur zwischen 600 °C und 1100 °C hergestellt wird, und wobei die Durchschlagspannung des Varistors (10) durch präzise Steuerung der Korngröße der Kernstruktur (14) und/oder Steuerung der Dicke oder des Isolationswiderstands der Schalenstruktur (12), welche die Isolationsschicht bildet, angepasst wird.

6. Verfahren nach Anspruch 5 zur Herstellung eines mehrschichtigen Varistor (10), umfassend:
a) Auswählen von pulverförmigen Materialzusammensetzungen (11) als Rohmaterial, die jeweils eine Kern-Schalen-Mikrostruktur aufweisen, wobei ein Korn, das eine Kernstruktur (14) bildet, aus dem leitenden oder halbleitenden Material besteht und eine Schalenstruktur (12), die um die Oberfläche des Korns der Kernstruktur (14) gewickelt ist, um eine Isolationsschicht zu bilden, aus Glasmaterial besteht;
b) Mischen der pulverförmigen Materialzusammensetzungen (11) mit einem geeigneten Bindemittel, Dispergiermittel, Weichmacher und organischen Lösungsmittel, um ein Pastenmaterial zu bilden;
c) Herstellen eines Grünbandes aus dem Pastenmaterial durch Foliengießen;
d) Stapeln einer vorgegebenen Anzahl von Grünbändern, auf die eine innere Elektrode (21) aufgedruckt ist, auf solche Weise, das Enden der inneren Elektroden (21) abwechselnd erscheinen;
e) Sintern der gestapelten Grünbänder bei einer Temperatur zwischen 600 °C und 1100 °C,
f) wobei die Durchschlagspannung des Varistors (10) bestimmt wird bei Schritt a) durch präzises Steuern von entweder der Größe der Kernstruktur (14) oder der Dicke der Glasschicht der Schalenstruktur (12) der pulverförmigen Materialzusammensetzungen (11), und/oder bei Schritt c) durch präzises Steuern der Dicke der jeweiligen Grünbänder in einem Bereich zwischen 15 µm und 200 µm.

7. Mehrschichtiger Varistor (10), der durch das Verfahren nach Anspruch 6 hergestellt wird, wobei in einem gesinterten Keramikkörper (20), der aus den pulverförmigen Materialzusammensetzungen (11) besteht, eine Glasmenge von mehr als 20 % enthalten ist.

8. Mehrschichtiger Varistor (10) nach Anspruch 7, wobei das leitende Material aus der Gruppe gewählt wird, die aus Fe, Al, Ni, Cu, Ag, Au, Pt, Pd und einer Legierung daraus besteht, und das halbleitende Material aus der Gruppe gewählt wird, die aus ZnO, SrTiO₃, BaTiO₃, SiC, TiO₂, SnO₂, Si und GaAs besteht.

## Revendications

1. Composition de matériau pulvérisée (11) pour une varistance (10) comprenant :
un conducteur en métal, un oxyde métallique semi-conducteur ou un matériau semi-conducteur ; et
un matériau en verre ;
**caractérisé en ce que**
la composition de matériau pulvérisée a une microstructure noyau-enveloppe, un grain formant une structure de noyau (14) étant faite en conducteur en métal, un oxyde métallique semi-conducteur ou un matériau semi-conducteur mentionné et une structure en enveloppe (12) enveloppée autour de la surface du grain de la structure en noyau (14) pour former une couche isolante étant faite en matériau en verre mentionné.

2. Composition de matériau selon la revendication 1, le conducteur en métal étant un alliage ou une combinaison de deux alliages ou plus ou une combinaison d'alliages de métaux sélectionnés dans le groupe contenant Fe, Al, Ni, Cu, Ag, Au, Pt et Pd.

3. Composition de matériau selon la revendication 1, le matériau semi-conducteur étant l'un des éléments ou une combinaison de deux éléments ou plus sélectionnés dans le groupe contenant ZnO, SrTiO₃, BaTiO₃, SiC, TiO₂, SnO₂, Si et GaAs.

4. Composition de matériau selon l'une des revendications 1, le matériau en verre étant sélectionné dans le groupe contenant le verre de silicate, le verre à base de bore, le verre en alumine et silice, le verre de phosphate et le verre de plomb.

5. Procédé pour fabriquer une varistance faite en composition de matériau pulvérisée (11) selon la revendication 1, la varistance (10) étant faite par frittage de la composition de matériau (11) à une température entre 500°C et 1100°C et la tension de rupture de la varistance (10) étant ajustée en contrôlant précisément la taille du grain de la structure en noyau (14) et/ou en contrôlant l'épaisseur ou la résistance d'isolement de la structure en noyau (12) qui forme la couche d'isolation.

6. Procédé selon la revendication 5 pour fabriquer une varistance en plusieurs couches (10) comprenant :
a) sélection de compositions de matériaux pulvérisés (11) comme matériau brut, chacune contenant une microstructure noyau-enveloppe, un grain formant une structure de noyau (14) étant faite en matériau conducteur ou semi-conducteur et une structure en enveloppe (12) enveloppée autour de la surface du grain de la structure en noyau (14) pour former une couche isolante étant faite en matériau en verre ;
b) mélange desdites compositions de matériaux pulvérisés (11) avec un liant approprié, un dispersant, un plastifiant et un solvant organique pour former un matériau en pâte ;
c) production d'un ruban vert fait en matériau en pâte par moulage par raclage ;
d) empilage d'un nombre prédéterminé de rubans verts ayant une électrode intérieure (21) imprimée dessus de telle manière que les extrémités des électrodes intérieures (21) apparaissent en alternance ;
e) frittage des rubans verts empilés à une température entre 600°C et 1100°C,
f) la tension de rupture de la varistance (10) étant conçue
à l'étape a) en contrôlant précisément soit la taille de la structure en noyau (14) ou l'épaisseur de la couche en verre de la structure en enveloppe (12) des compositions de matériaux pulvérisées (11) et/ou
à l'étape b) en contrôlant précisément l'épaisseur de chaque ruban vert à l'intérieur d'une plage entre 15 µm et 200 µm.

7. Varistance à plusieurs couches (10) produite par le procédé de la revendication 6, un corps céramique fritté (20) construit à partir des compositions de matériaux pulvérisées (11) contenant une quantité de verre supérieure à 20%.

8. Varistance à plusieurs couches (10) selon la revendication 7, le matériau conducteur étant sélectionné dans le groupe contenant Fe, Al, Ni, Cu, Ag, Au, Pt et Pd et les alliages de ceux-ci et le matériau semi-conducteur étant sélectionné dans le groupe contenant ZnO, SrTiO₃, BaTiO₃, SiC, TiO₂, SnO₂, Si et GaAs.
